

1

2,825,697

## METHOD OF AND SOLUTION FOR THE SURFACE TREATMENT OF ALUMINUM

John A. Carroll, Philadelphia, and Nelson J. Newhard, Jr., Oreland, Pa., assignors to American Chemical Paint Company, Ambler, Pa., a corporation of Delaware

No Drawing. Application August 5, 1954  
Serial No. 448,164

2 Claims. (Cl. 252—389)

This invention relates to the art of increasing the corrosion resistance of aluminum and alloys thereof in which aluminum is the principal or predominant ingredient. In the following disclosure the word "aluminum" is to be understood as including such alloys.

As is well known, unprotected aluminum surfaces are susceptible to corrosion and in an effort to overcome this tendency it has been customary in the art to deliberately produce an oxide film on the aluminum surface which, if properly formed by either chemical or electrical means, will serve as an effective barrier between the basic metal and the corrosive influences of the atmosphere. However, processes of the kind just referred to are open to certain objections. For instance, chemical processes for the production of an oxide film usually produce a film which has a distinctly mottled appearance. Therefore, where it is necessary or desirable to preserve a uniform metallic appearance, electrochemical treatments have been resorted to because of their ability to yield a protective oxide film which does not necessarily substantially alter the physical appearance of the surface. Such electrochemical processes, however, have the disadvantage of requiring large amounts of electrical equipment. In addition, they are time consuming and relatively expensive.

With the foregoing in mind, the principal object of our invention is the provision of a method and solution for the treatment of aluminum surfaces whereby they may be rendered highly passive and corrosion resistant without discoloring or in any way marring the surface and without using cumbersome electrolytic equipment.

Another object of the invention is to provide a process of the character described which is so simple and effective that it can be used by relatively unskilled personnel and under a wide variety of conditions—in other words, a process which is relatively uncritical as to the manner and means by which it is carried out.

Still another object of the invention is the provision of a process for effecting the foregoing objectives without the necessity of removing from the surface of the aluminum any pre-formed naturally occurring oxide film which may be present.

As indicated, our improved process is in the nature of a passivating procedure which does not appreciably alter the appearance of the aluminum surface and how the foregoing objects together with such other objects as may appear hereinafter or are incident to our invention are attained will now be described.

We have discovered that aluminum surfaces can be passivated and their corrosion resistance greatly increased, and this without marring or discoloring the surface, if they are treated with dilute aqueous acid solutions containing as their principal and essential ingredients some "fluorine-bearing compound" and a source of hexavalent chromium in accordance with the following teachings.

By the term "fluorine-bearing compound" we mean a complex fluoride such as fluosilicic acid, fluoboric acid, fluozirconic acid, fluostannic acid, fluotitanic acid and

2

the soluble salts of any of them. By the term "hexavalent chromium," we mean chromic acid ( $\text{CrO}_3$ ) or its soluble salts such as ammonium dichromate, potassium dichromate, sodium chromate, etc.

5 The amounts of these ingredients present in the solution is important. Of the fluorine-bearing compound there should be present in the bath between 0.1 and 1.0 gram per liter calculated as fluorine. At concentrations of less than 0.1 gram per liter there is a marked falling off in the effect produced by the solution. At concentrations greater than 1 gram per liter there is a tendency to produce a visible coating upon the aluminum.

As for the quantity of hexavalent chromium in the bath there should be from 0.4 gram to 4 grams per liter 15 calculated as  $\text{CrO}_3$ . At concentrations of less than 0.4 gram very little effect is produced and when the concentration exceeds 4 grams per liter there is a tendency for the solution to produce a visible coating on the aluminum.

The pH of the treating solution is also important. 20 Preferably the fluorine-bearing compound and the hexavalent chromium should be present in the solution in such proportions and amounts as to yield a pH of from 2.0 to 4.0. At pH's below 2.0 there is a tendency for the solution to produce visible coatings on the aluminum 25 and at pH's above 4.0 the surface does not appear to become particularly passive. If the sources of fluorine-bearing compound and of hexavalent chromium used in preparing the solution are of such nature that the solution does not have a pH as specified it may be adjusted, if too 30 high, by the addition of a suitable quantity of some mineral acid such as nitric acid or hydrochloric acid. On the other hand, if the pH is too low, it can be raised by proper additions of an alkali such as sodium hydroxide, ammonium hydroxide, etc.

35 As for the time of treatment, the temperature of the bath and the manner in which the solution is contacted with the surface, we have found no particular limitations that seem to be important. A minimum treating time is usually in the neighborhood of one minute but longer periods of treatment have also been employed with excellent 40 results. In general, it would appear that best results are to be attained by allowing the solution to act upon the surface for from one to two minutes where the temperature of the bath is maintained at approximately 160° F.

45 However, the matter of temperature does not appear to be in any way critical because we have obtained excellent results anywhere from ordinary living-room temperatures (i. e., approximately 68° to 78° F.), all the way up to practically the boiling point of the solution.

50 The manner in which the solution is brought into contact with the surface is also capable of considerable variation without in any way hindering the results to be obtained. For example, the article to be treated may be immersed in the bath or the solution may be applied to the surface as a spray or it may be wiped with a cloth dampened with the solution or by any other means which insures thorough wetting of the surface. Where the solution is applied by some wiping expedient it is allowed to dry on the surface but regardless of these various factors we have learned by experience that best results are generally obtained if the following "rule of thumb" method of preparing the treating bath is employed. When the concentration of fluorine-bearing compound is relatively 55 low then the concentration of hexavalent chromium should also be relatively low and, conversely, when the concentration of fluorine-bearing compound is high the concentration of hexavalent chromium also should be relatively high. Another general rule which is useful

60 to observe is that where the solution is used hot we prefer a more dilute solution and, conversely, where the solution is to be applied at a relatively cool temperature,

i. e., room temperature, then a more concentrated solution is preferred.

By way of specific example within the teachings above set forth, suitable treating solutions useful in the process of the present invention are as follows:

*Example 1*

|                              | Grams |
|------------------------------|-------|
| Chromic acid                 | 0.46  |
| Potassium zirconium fluoride | 0.29  |
| Water, to make 1 liter.      |       |

*Example 2*

|                             | Grams |
|-----------------------------|-------|
| Chromic acid                | 2     |
| Potassium titanium fluoride | 1.4   |
| Water, to make 1 liter.     |       |

The material of Example 1 is ideally adapted to treat aluminum in an immersion process and we have secured excellent results by immersion for from one to two minutes with the temperature of the bath maintained at approximately 160° F. Following this, the article is removed, excess liquid is rinsed off with ordinary tap water and the surface dried.

It should be pointed out that the surface to be treated should be relatively clean although it is not necessary to remove any natural light oxide film which may be present unless such film is of a nature which is aesthetically unappealing or unsatisfactory, it being understood in this connection that the present invention is primarily concerned with a passivating procedure which leaves the surface substantially colorless or unchanged. In other words, naturally occurring oxide films are not deleterious, *per se*, which, of course, is a distinct advantage over other procedures heretofore employed which first require the removal of any natural oxide film before the treatment is applied. As an actual matter of fact, for some reason which we do not fully understand, the amount of passivation and corrosion resistance secured by our invention seems to be markedly enhanced in situations where a naturally occurring oxide film is left on the surface at the time that our solution is applied thereto.

The material of Example 2 is ideally adapted for application to the surface by means of brush, rags, etc. and we have found that by using a material such as exemplified by Example 2, exceedingly good passivation is achieved if the solution is permitted to act upon the surface for from one to two minutes at room temperature although no harm is done if the material is permitted to dry upon the surface should this be desirable or convenient. However, if the solution is permitted to dry on the surface the aluminum may be stained somewhat due to the hexavalent chromium powder which will be found lying loose on the surface.

Spraying procedures for applying the solution may also be employed but in such procedures as well as in the foregoing procedures length of time and the temperature of the bath do not seem to be too critical although from the standpoint of economy in cost reasonably short

periods of exposure to the effects of the solution and relatively low temperatures are to be preferred.

Somewhat surprisingly, the invisible passivation which we secure is obtained by utilizing what may be described as an "activating solution" which definition is employed because of the peculiar properties imparted to the aluminum surface by the process which we have developed. For example, if a previously deoxidized aluminum surface is treated according to our invention it will exhibit, immediately after the treatment, an extremely low electrical surface contact resistance. This bespeaks an "activated" surface toward oxidation. However, the electric contact resistance of a surface treated in accordance with our invention rapidly increases after a short time lapse and at a much greater rate than it does on a deoxidized but otherwise untreated aluminum surface. Surfaces treated in accordance with our invention, despite their apparent lack of any visible protective coating, have successfully withstood 168 hours exposure to a salt fog test conducted in accordance with U. S. Government specification Q-Q-M-151a. As contrasted with this showing, previously deoxidized but otherwise untreated aluminum surfaces even after a lapse of time during which a naturally occurring oxide film will form, exhibit far less corrosion resistance when exposed to the same salt fog test, a typical example being approximately 24 hours before substantial break-down occurs.

We claim:

1. The method of increasing the corrosion resistance of an aluminum surface without changing its appearance which consists in treating the surface with an aqueous acid solution consisting essentially of hexavalent chromium and a soluble complex fluorine-bearing compound, the amount of hexavalent chromium being from 0.4 gram to 4 grams per liter calculated as  $\text{CrO}_3$  and the amount of fluorine-bearing compound being from 0.1 gram to 1.0 gram per liter calculated as fluorine and the pH of the solution being from 2.0 to 4.0.

2. The method of claim 1 wherein the hexavalent chromium is chosen from the group consisting of chromic acid ( $\text{CrO}_3$ ) and its soluble salts and the fluorine-bearing compound is chosen from the group which consists of fluosilicic acid, fluoboric acid, fluozirconic acid, fluostannic acid, fluotitanic acid and the soluble salts thereof.

References Cited in the file of this patent

UNITED STATES PATENTS

|    |           |                 |                |
|----|-----------|-----------------|----------------|
| 50 | 2,494,910 | Spruance        | Jan. 17, 1950  |
|    | 2,499,231 | Stareck         | Feb. 18, 1950  |
|    | 2,563,431 | Spruance        | Aug. 7, 1951   |
|    | 2,568,936 | Spruance        | Sept. 25, 1951 |
|    | 2,655,439 | Floersch        | Oct. 13, 1953  |
| 55 | 2,678,291 | Spruance et al. | May 11, 1954   |
|    | 2,727,841 | Chester         | Dec. 20, 1955  |
|    | 2,762,731 | Heller          | Sept. 11, 1956 |
|    | 2,798,829 | Newhard et al.  | July 9, 1957   |
|    | 2,798,830 | Newhard et al.  | July 9, 1957   |